

# United States Patent Office

2,970,903

Patented Feb. 7, 1961

1

2,970,903

## ALLOY STEEL HAVING SURFACE FREE FROM ALLIGATORING

Cedric G. Mickelson, Gary, Ind., and Charles D. Asherman, Chicago, Ill., assignors to American Steel Foundries, Chicago, Ill., a corporation of New Jersey

No Drawing. Filed Aug. 14, 1958, Ser. No. 755,070

8 Claims. (Cl. 75—123)

This invention relates to alloy steel and more particularly to alloy steel castings having good wear resistance, high impact strength and a smooth, defect free surface.

Alloy steels have been developed having high impact values, particularly at low temperatures, and also having such properties as toughness, corrosion and wear re-

must be present, as an addition to the molten metal, in the amount of at least about 0.35% by weight of the molten metal. These percentages are critical and it should be noted that all three constituents, namely, silicon, aluminum and rare earth, must be utilized in at least the percentages indicated.

The rear earth metal addition referred to herein, is intended to mean any of the rear earth metals, but particularly combinations thereof including lanthanum, cerium, praseodymium and neodymium, though other combinations are equally effective.

The following typical heats of tough, high impact strength, alloy steels are given by way of example to illustrate the effect of varying the percentages of silicon, aluminum and rare earth metals on the surface condition of castings poured from the heats. The percentages given for aluminum and the rare earth metals represent an addition for deoxidation purposes, it being understood that the steel castings resulting from the heats will contain only the deoxidation residue.

| Heat No. | C   | Mn   | Si  | P    | S    | Cr   | Mo  | Ni   | B     | Addition |                   |
|----------|-----|------|-----|------|------|------|-----|------|-------|----------|-------------------|
|          |     |      |     |      |      |      |     |      |       | Al       | Rare Earth Metals |
| 1        | .21 | 2.08 | .53 | .015 | .017 | 1.03 | .57 | .98  | .0031 | .125     | .25               |
| 2        | .27 | 1.99 | .36 | .016 | .012 | 1.03 | .65 | 1.05 | .0028 | .125     | .35               |
| 3        | .21 | 2.13 | .83 | .019 | .018 | 1.07 | .64 | 1.05 | .0027 | .125     | .10               |
| 4        | .25 | 2.07 | .63 | .011 | .012 | 1.00 | .62 | 1.06 | .0024 | .125     | .35               |

sistance, and weldability. However, satisfactory castings utilizing these alloy steels have been produced only in relatively thin sections. When castings having sections of about four inches or greater in thickness have been poured, they have been subject to surface defects commonly called and referred to hereinafter as alligatoring.

Alligatoring may be defined as a surface condition characterized by random, irregular cracks, of varying depth, and resembling to a great extent the appearance of cracked, parched earth. Thus surface condition is believed to be caused by excessive oxidation at the surface grain boundaries where oxidation occurs more rapidly than at other areas of exposed surface. The condition is accentuated when the rate of cooling is decreased because in this instance, there is a greater length of time for the oxidation to occur. Factors which particularly contribute to the formation of alligatoring are casting sections of approximately four inches and upward in thickness and also the pouring of the alloy steel in sand molds, both of which have the effect of greatly reducing the rate of cooling.

The steel alloys which have the best impact and toughness characteristics but which also give the most trouble with respect to alligatoring when cast with sections in the range of four inches and thicker are those containing, as alloy constituents, one or more of the group including manganese, chromium and nickel in the following proportions:

Mn, 1.50 to 2.50%; Cr, 0.75 to 3.00%; and Ni, 0.75 to 3.50%.

It has been found, according to the present invention, that the surface defect known as alligatoring can be completely eliminated from alloy steel castings of the type referred to herein even when these castings are poured in sand molds and are cooled slowly. The invention contemplates the inclusion or addition of silicon, aluminum and rare earth metals in minimal quantities. Specifically, silicon must be present in the amount of at least about 0.60%; aluminum must be present, as an addition to the molten metal, in the amount of at least about 0.10% by weight of the molten metal; rare earth

35 The metal from these heats was poured into green sand molds using silica sand as the molding material. The test bars comprised sections varying from about four inches to about eight inches in thickness. The castings were not shaken out until the following day at which time they had almost reached room temperature. It should be noted, however, that the shake-out temperature has no great effect on the quality of the castings.

40 Heat No. 1 shows a silicon content and a rear earth metal addition below the minimal quantities. Heat No. 2 illustrates an attempt to compensate for a low silicon content by a high rare earth metal addition. Heat No. 3 illustrates an attempt to compensate for a low rare earth metal addition by an extremely high silicon content. The castings from heats No. 1, 2, and 3 had surfaces with moderately heavy alligator skin. However, the outer surface of the castings produced from heat No. 4 was entirely free from surface defects and no evidence of alligatoring was present.

55 The minimal silicon content of 0.60% together with the addition to the molten metal of at least about 0.10% aluminum and at least about 0.35% rare earth have been found to eliminate alligatoring from casting surfaces in alloys having the following components in the ranges indicated: about 0.25 to 0.50% carbon; nil to about 0.025% sulphur; nil to about 0.025% phosphorus; about 0.75 to about 3.00% chromium; about 0.50 to 0.65% molybdenum; and about 0.0005 to about 0.005% boron.

60 We claim:

1. A high impact, wear resistant low alloy steel for heavy section castings characterized by a surface free from alligatoring, said alloy comprising silicon in the amount of at least 0.60%, said alloy steel being deoxidized by the addition to the molten metal of at least about 0.10% aluminum and at least about 0.35% rare earth, based on the weight of molten metal.

65 2. A high impact, wear resistant low alloy steel for heavy section castings characterized by a surface free from alligatoring, said alloy comprising silicon in the amount of at least 0.60%, said alloy steel being deoxidized by the addition to the molten metal of at least

about 0.10% aluminum and at least about 0.35% rare earth, based on the weight of molten metal.

3. A high impact, wear resistant low alloy steel for castings having minimum section of about four inches and characterized by a surface free from alligatoring, said alloy having a silicon content of at least about 0.60%, said alloy being deoxidized by the addition to the molten metal of at least about 0.10% aluminum and at least about 0.35% rare earth, based on the weight of molten metal.

4. A high impact, wear resistant low alloy steel for castings having sections of about four to eight inches, characterized by a surface free from alligatoring, said alloy containing silicon in the amount of at least 0.60%, and the residue from the treatment of the molten metal with at least 0.10% aluminum and at least 0.35% rare earth, based on the weight of molten metal.

5. A high impact, wear resistant alloy steel for castings having sections of about four to eight inches, and characterized by a surface free from alligatoring, said alloy containing about 1.50 to 2.50% manganese, about 0.75 to 3.00% chromium, about 0.75 to 3.50% nickel, at least 0.60% silicon, and the residue from the treatment of the molten metal with at least 0.10% aluminum and at least 0.35% rare earth based on the weight of molten metal.

6. An alloy steel for castings having a minimum section thickness of about four inches and having a surface substantially free from defects, said alloy including at least one element selected from the group consisting of: manganese 1.50 to 2.50%; chromium 0.75 to 3.00%,

and nickel 0.75 to 3.50%, said alloy having a silicon content of at least about 0.60%, said alloy being deoxidized by the addition to the molten metal of at least 0.10% aluminum and at least about 0.35% rare earth, based on the weight of molten metal.

5 7. An alloy steel for castings having a minimum section thickness of about four inches and having a surface substantially free from defects, said alloy being composed of about 0.75 to 9.0% of the group consisting of manganese, chromium and nickel, and at least about 0.60% silicon, said alloy being deoxidized by the addition to the molten metal of at least 0.10% aluminum and at least about 0.35% rare earth, based on the weight of molten metal.

10 8. A steel alloy for castings having a minimum section thickness of about four inches and a surface substantially free from defects, said alloy steel being composed of about 0.25 to 0.50% carbon, up to about 0.025% sulphur, up to about 0.025% phosphorus, about 0.75 to 20 3.00% chromium, about 1.50 to 2.50% manganese, about 0.75 to 3.50% nickel, about 0.50 to 0.65% molybdenum, about 0.0005 to 0.005% boron, at least about 0.60% silicon and the residue from the addition in the molten state of at least 0.10% aluminum and at least about 25 0.35% rare earth based on the weight of molten metal, the balance iron.

References Cited in the file of this patent

UNITED STATES PATENTS

30 2,823,992 Bolkcom et al. \_\_\_\_\_ Feb. 18, 1958  
2,861,908 Mickelson et al. \_\_\_\_\_ Nov. 25, 1958

UNITED STATES PATENT OFFICE  
CERTIFICATE OF CORRECTION

Patent No. 2,970,903

February 7, 1961

Cedric G. Mickelson et al.

It is hereby certified that error appears in the above numbered patent requiring correction and that the said Letters Patent should read as corrected below.

Column 1, line 41, for "Thus" read -- This --; column 2, lines 7, 8, and 40, for "rear", each occurrence, read -- rare --; column 4, line 13, for "base don" read -- based on --.

Signed and sealed this 14th day of November 1961.

(SEAL)

Attest:

ERNEST W. SWIDER  
Attesting Officer

DAVID L. LADD  
Commissioner of Patents  
USCOMM-DC